

G. H. HADFIELD AND A. E. BAWTREE.  
PROCESS FOR TREATING POROUS VESSELS.  
APPLICATION FILED OCT. 15, 1918.

1,306,375.

Patented June 10, 1919.



Inventors  
and G. H. Hadfield  
A. E. Bawtree

By their Attorneys  
Baldwin & Wright

Witnesses

*John Carter*

# UNITED STATES PATENT OFFICE.

GEORGE HUGH HADFIELD, OF MITCHAM, AND ALFRED EDWIN BAWTREE, OF SUTTON, ENGLAND.

## PROCESS FOR TREATING POROUS VESSELS.

1,306,375.

Specification of Letters Patent. Patented June 10, 1919.

Application filed October 15, 1918. Serial No. 258,307.

To all whom it may concern:

Be it known that we, GEORGE HUGH HADFIELD, a subject of the King of Great Britain, residing at Hadfields (Merton) Limited, 5 Western Road, Mitcham, Surrey, England, varnish manufacturer, and ALFRED EDWIN BAWTREE, a subject of the King of Great Britain, residing at 7 Manor Park road, Sutton, Surrey, England, have invented a new 10 and useful Improved Process for Treating Porous Vessels, of which the following is a specification.

This invention relates to a process for treating the inner walls of vessels composed 15 or more or less porous material with a suitable fluid which dries or sets after a period. The process is particularly applicable to the treatment of vessels composed partly or wholly of paper or cardboard.

20 Various difficulties arise in making a thoroughly impervious vessel. Thus the interior portions of the vessel do not usually consist of perfectly continuous surfaces but are broken up by pits or fissures due to the 25 method of manufacture. For example, one form of cylindrical package has a spiral crack or groove around its interior where two strips of cardboard butt. If the interior surfaces of such vessels are merely 30 flowed over or lightly brushed over with a fluid composition, such composition merely bridges across the fissures or grooves and upon drying cracks leaving them quite unprotected.

35 In the accompanying drawing,

Figure 1 shows a vertical section of a vessel of porous material constructed and treated according to our invention.

40 Figs. 2, 3 and 4 illustrate the steps of one way of carrying out our invention.

Fig. 2 shows how a vessel of porous material formed by spirally winding paper or the like has its opposite ends dipped in proofing material.

45 Fig. 3 illustrates how the vessel treated in the manner indicated in Fig. 2 has a bottom applied to one end and a ring, forming part of the closure, applied to the other end.

Fig. 4 shows the next step in the process 50 wherein the interior of the vessel and the joints, fissures, etc., are coated and filled with proofing material.

Fig. 5 illustrates a machine which may be employed for rotating the vessel during the 55 process of coating or proofing the interior thereof.

According to this invention a quantity of a protective fluid or composition which has little or no penetrative power into the substance of the vessel treated, is placed in the 60 vessel and is then spread over every detail of the contour of the interior surface by the action of centrifugal force. The vessel must be rotated at such a speed that if its axis be horizontal centrifugal force shall at least 65 counteract the force of gravity in portions of surface which are for the time being vertically above the axis of rotation as in this case the coating material will be driven so strongly into the imperfections in the surface 70 as to cause the coating to accurately follow every detail of the contour of the surface. At the same time it is evident that the axis of rotation need not necessarily be truly horizontal but may be inclined to any convenient angle. 75

If the rotation be at too low a speed the coating fluid or composition would flow by gravity over the entire surface in the manner already known in such operations as in the 80 pitching of barrels, but such coating would not be reliable. It is important that the fluid should accurately follow the surfaces of the imperfections in the walls of the vessel in the manner described. It is also important 85 that this penetration of imperfections should not be confounded with the soaking in by capillary attraction or impregnation brought about in any other manner. It is essential for securing the objects of our invention that 90 at least a portion of the fluid should stand out upon the surface. The action of centrifugal force does not prevent a suitable composition from doing this, but it causes 95 a film of composition to follow the surfaces of even the deepest imperfections.

The period during which the vessel to be treated is rotated depends upon the quantity of fluid in the vessel; if a small quantity of fluid be employed, rotation is merely continued till it is evenly distributed; if a larger amount be used, rotation must be continued till it has become set and no longer fluid. In this latter case there is no limit to the thickness of composition which can be spread 100 upon the surface at a single operation.

The process may be carried out with the aid of any known mechanism for causing the necessary rotation of the vessel which should combine the necessary speed with 110 great accuracy of rotation. This last point is one of great importance. If, for example,

a container is receiving a coating of fluid one sixteenth of an inch thick, but one side is one sixteenth of an inch farther from the center of rotation than the other, this side will receive the whole of the supply of coating material except such small quantity as may adhere to the portions nearer to the center of rotation by the action of capillary attraction.

The fluid or composition employed in the process depends upon the use to which the vessels are to be put and the composition forms no part of this invention as the use of colloids such as glue and gelatin mixed with hardening agents are known for this purpose as are also various waxes and the like and compositions consisting of rosin, linseed oil driers and turpentine, which will set hard or nearly so when cold.

With some vessels and especially when a small quantity of fluid is placed in the vessel it is necessary in order to produce a satisfactory result to subject the vessel to a preliminary treatment which has for its object the efficient sealing of the joints between the ends and sides of the vessel. To perform this operation we treat one or both of the surfaces to be united with a composition possessing similar properties to that which we use for rendering the main portion of the surface of the vessel impervious and make the joints while such composition is still in a more or less soft state. By this means any small fissures or imperfections occurring in the operation of joining the portions of the vessel together are closed whereas if the coating of composition had been allowed to become hard before making the joints, there would be the same possibility of leakage as exists when the portions of a tin canister are merely bent together.

The following are specific examples of applications of our invention:—

1. A canister has a tin bottom and for its top a tin ring into which fits a lever lid, the sides being composed of layers of paper. It is desired to render such a vessel suitable for containing a paint the ingredients of which include oil and turpentine spirit. A suitable protecting composition would be a 10% solution of gelatin, the cardboard having been previously treated with a hardening agent such as a saturated solution of alum.

Each end of the cardboard tube which is to form the sides of the vessel is first by any suitable mechanism coated at the edges of the ends and to a short distance along each end of the interior surface. While the composition is still wet the tin ends are spun on in the ordinary manner.

60 The canister is placed in a suitable chuck and a quantity of the coating composition poured in; the chuck is then revolved at a sufficiently high speed to produce the phenomenon of the counteraction of gravitation by centrifugal force if the axis of rotation

be horizontal in the manner above referred to. This preliminary treatment of the end of the vessel before spinning on tin ends may however be dispensed with if sufficient composition is employed.

2. A canister similar to that employed in example No. 1 is treated as in that example so far as placing the tin bottom and the tin ring is concerned. It is now placed in a chuck and supplied with its quantum of composition, by means of a brush charged with the coating fluid: a coating is thus distributed over the surface to be proofed, either before or while the vessel is rotating. Rotation is then continued for a sufficient time and at a sufficient speed to produce the close fitting film secured by the action of centrifugal force.

3. A tube composed wholly of cardboard and provided with a cardboard shut over lid is to be used for holding adhesive composed of dextrin and water. The coating composition to be employed consists of rosin, 3 parts, linseed oil containing 1% of dissolved litharge 1 part and turpentine 1 part and is of such a consistency as to be barely fluid when cold.

The bottom cap is first placed upon a revolving support and a little hot composition poured into it. Centrifugal force distributes the composition over the bottom and up the sides of the cap.

The cardboard tube is then pressed into the cap, a supply of melted composition is poured in, the mouth of the tube is closed with a conical stopper and the tube rapidly rotated until the composition is first evenly distributed and then sets, partly by cooling and partly by the absorption by the porous walls of the spirit and oil which it contains.

Referring again to the accompanying drawings, we have illustrated in Fig. 5 a machine which may be employed for rotating the vessel during the proofing process. As there shown the container A is gripped by the jaws B of a self-centering chuck C, attached to a shaft or spindle D, turning in bearings E, mounted in an ordinary lathe head F. The shaft or spindle is provided with a pulley G, to which power may be applied for rotating it. Any other suitable machines for this purpose may, however, be employed.

Referring to Fig. 1, we have shown a vertical section of a vessel or container treated in accordance with our improvements. *a* indicates the body of the container, which in this instance is made of spirally wound paper or cardboard. In all such cases there is usually present a groove, crack or fissure *b* on the interior of the vessel. *c* indicates the bottom closure. In this instance it consists of a disk of tin, having its peripheral portion *c'* bent around the lower end of the body portion *a*. *d* indicates a ring of metal ap-

plied to the upper end of the container, its peripheral portion  $d'$  being bent around the end of the body  $a$ . This form of container is well known and is used by us for 5 purposes of illustration only, it being understood that our improvements may be applied to containers of other kinds. The body portion  $a$ , made of paper, cardboard or other porous material and having the characteristics before mentioned, is preferably first 10 dipped into suitable proofing material, in a way before described, in such a way as to cause its lower end to receive an annular coating  $x$  of the proofing material, and the 15 opposite end or top of the body  $a$  is also preferably treated in the same way to receive an annular coating  $x'$ . (The product of this stage of manufacture is represented in Fig. 2.) The next step in the preferred 20 process is to apply the bottom  $c$  and the top ring  $d$ , in the manner indicated in Fig. 3. The purpose of applying the proofing material  $x$ ,  $x'$  is to insure the closing of the joints at both top and bottom when the vessel is rotated in the manner before described. 25 Without such preliminary treatment there is liability of the joints not being completely sealed unless the centrifugal treatment is continued for a considerable time.

30 Fig. 4 illustrates the completed vessel after the proofing material has been applied centrifugally in the manner hereinbefore explained. This proofing material, which is indicated at  $y$ , it will be observed, completely covers the interior of the paper or porous portions of the vessel, and it will also be observed that the material enters the grooves  $b$ , as indicated at  $z$ . It is made to 35 so enter the grooves by the centrifugal action before explained. Without such treatment the proofing material would merely bridge the grooves and would be liable to crack or open along the grooves, and thus produce leakage. It will also be observed that by the centrifugal action mentioned the 40 joint of the bottom  $c$  with the body of the container is completely closed, the proofing 45

material  $y$  uniting with the material  $x$  to close the joint and thus prevent any leakage that might occur unless special provision 50 was made to prevent it.

As before specified, after the body of the vessel is prepared in the manner indicated in Fig. 3, it is supplied with a suitable amount of proofing material and is then 55 held by rotating mechanism in the manner indicated in Fig. 5 so as to rotate about a horizontal axis with great accuracy for the reasons before specified.

It will be understood that a suitable closure or lid may be applied to the ring  $d$ . It 60 will also be understood that we do not intend to limit our invention to the preliminary treatment before specified as it is not in all cases necessary.

We are aware that it has been proposed to 65 impart rotation to cartridges while their interiors are being varnished with a brush but it is clear that in the treatment of these articles the action of centrifugal force is 70 not made use of. Such force, owing to its great power of uniformly spreading a fluid would cause the varnish to flow over the portion of the tube which has at great pains 75 been cleaned with a wiper for the reception of the bullet.

What we claim is:—

A process of applying a liquid coating composition capable of hardening, to the interior surface of a receptacle of which the inner wall is made of a somewhat pervious material having cracks or fissures therein, such process comprising rotating the receptacle, with such coating composition therein, at such a rapid rate of speed that the said 80 coating composition is spread out in the form of a coating on the interior of said receptacle, and forced into said cracks and fissures, substantially as specified.

In testimony that we claim the foregoing 85 as our invention, we have signed our names this 19th day of September, 1918.

GEORGE HUGH HADFIELD.  
ALFRED EDWIN BAWTREE.